



US007585454B2

(12) **United States Patent**  
Noga et al.

(10) **Patent No.:** US 7,585,454 B2  
(45) **Date of Patent:** Sep. 8, 2009

(54) **PROCESS OF AND APPARATUS FOR  
MAKING AN INSULATION PRODUCT**

(75) Inventors: **Michael J. Noga**, Oakville (CA); **David Warren Arseneau**, Burlington (CA); **John D. Ireland**, Burlington (CA); **William Malcolm Worden**, Oakville (CA); **Zhiyong Fu**, Hamilton (CA); **Reginald A. Cooke**, Burlington (CA); **Martin H. Beck**, Amherst, NH (US)

(73) Assignee: **RTICA, Inc.**, Haliburton, ON (CA)

(\*) Notice: Subject to any disclaimer, the term of this patent is extended or adjusted under 35 U.S.C. 154(b) by 831 days.

(21) Appl. No.: **10/490,396**

(22) PCT Filed: **Sep. 30, 2002**

(86) PCT No.: **PCT/US02/30995**

§ 371 (c)(1),  
(2), (4) Date: **May 5, 2004**

(87) PCT Pub. No.: **WO03/029535**

PCT Pub. Date: **Apr. 10, 2003**

(65) **Prior Publication Data**

US 2004/0232602 A1 Nov. 25, 2004

(51) **Int. Cl.**

**B29C 39/14** (2006.01)  
**B29C 43/22** (2006.01)

(52) **U.S. Cl.** ..... **264/555**; 264/638; 264/639;  
264/677; 264/556; 264/559

(58) **Field of Classification Search** ..... 264/555,  
264/342, 638, 639, 677, 556, 559, 112, 113,  
264/116, 118, 130, 131, 145, 148, 152, 157–160,  
264/171.1, 171.17, 241, 257, 258, 291, 288.4,  
264/297.4

See application file for complete search history.

(56) **References Cited**

**U.S. PATENT DOCUMENTS**

2,209,850 A \* 7/1940 Shand et al. ..... 156/148  
4,351,683 A \* 9/1982 Kusilek ..... 156/167  
5,582,905 A \* 12/1996 Beck et al. ..... 428/74  
5,958,322 A \* 9/1999 Thompson et al. .... 264/342 RE  
2004/0159658 A1 \* 8/2004 McLaughlin et al. ..... 220/4.21

\* cited by examiner

*Primary Examiner*—Christina Johnson

*Assistant Examiner*—Stella Yi

(74) *Attorney, Agent, or Firm*—Davis & Bujold, P.L.L.C.

(57) **ABSTRACT**

A method of producing a non-lofted fiber veil of an orientable polymer for the production of insulation, e.g. thermal, for blown-in applications, having X, Y and Z vector directions of the fibers comprising, melt blowing the polymer to form molten fibers, having molecules oriented along the length of the fibers, the X vector direction, placing the fibers on a roller spinning at a rate to provide additional orientation of the molecules of the fibers, displacing some said fibers into the Y vector direction, and cooling the fibers while on the roller to form the non-lofted fiber veil. Also included is the product of the method, a blown in insulation, intermediate products, an apparatus and a method of producing a product for blown-in installation.

**15 Claims, 8 Drawing Sheets**





FIG. 1



FIG.2



FIG.3



FIG.4



FIG.6

FIG.5



FIG. 7



FIG.8



FIG.9



FIG.10

## 1

PROCESS OF AND APPARATUS FOR  
MAKING AN INSULATION PRODUCT

This invention relates to a new apparatus and method for producing a new product useful as a blown in insulation and made of a orientable polymer (preferably heat setable), e.g. PET, and the new product itself.

## BACKGROUND OF THE INVENTION

Insulation products made from polymer fibers are not new as there are several products in the marketplace, however, most of these applications are for clothing apparel and the like. Blown-in insulation of homes and buildings generally use fiberglass or cellulose.

There are environmental hazards and inefficiencies using these other materials. For example, fiberglass and cellulose will break apart into fine particles when put through conventional blow-in insulation equipment. These fine particles are hazardous to human beings upon breathing large quantities thereof. In addition, both materials, fiberglass and cellulose, are inferior to polymer (specifically PET) fibers for performance in insulation value and other measurable physical characteristics (such as cycling through wet and dry conditions).

In the present invention polymer fiber is made by way of a preferred process generally called melt blowing. This method is known in the plastics converting industry as a method to form small diameter fibers. U.S. Pat. No. 5,582,905 assigned to the assignee of the present application discloses a method of making continuous fibers, collecting the fibers and making a batt (lofted in the z direction).

Fiber (and products) made from the melt blowing process have typically been limited by the properties generated from the melt blow process.

## OBJECT OF THE INVENTION

It is an object of the present invention to overcome the environmental disadvantages of the prior art blown in insulation and to provide an environmentally safe stable lofted polymer insulation having an insulation value superior to the prior art.

## SUMMARY OF THE PRESENT INVENTION

Products of the present invention typically are continuous fibers laid out in a thin web sheet (veil) in the X and Y directions with little or no loft (Z direction).

The new product of this invention disclosed herein is a non-lofted veil made from a fiber that, produced as a non-lofted veil with fibers in the X and Y direction, is processed to improve its properties and then is cut into short segments (1 to 30 mm long) compactly bundled for expansion on location. A significant portion of the fibers of these segments extend in the Z direction upon compaction. When the final product is made the fibers are substantially evenly dispersed into the X, Y and Z directions.

The present invention enhances the quality of the fiber and the end product (mass of fibers). Specifically, high levels of orientation (in fibers, it is generally monoaxial orientation) and crystallinity are the properties desired for fibers used in insulation product such as blown-in attic insulation. Products such as filtration media where the fibers are enclosed within a structure can utilize even smaller fibers.

Disclosed is a fiber product for blown-in insulation, made by way of several steps including orientation via the hot air

## 2

followed by quenching to lock in orientation. Additional orientation is added downstream to the fibers and web by way of further heating mechanical actions including crystallization of the oriented fiber. The fiber is oriented 3 (or more) times during the process under different conditions.

Specifically a controlled web (veil), essentially a 2 direction (X and Y) product, is produced in which the fibers are oriented twice in the X direction and then a fractional component of the oriented X direction is redirected to lay in the Y direction. This is accomplished by use of the hot air flow in the X direction and the turbulent currents created by that flow and presence of a mechanical roller.

Nodal points (where 2 fibers cross each other and fast with each other at that point) are created in the X and Y vector (X=machine direction, Y=cross machine direction) to create more and stronger Z direction fiber in the blown-in product.

Following this the cutting and compaction of the web directs a substantial portion of the fibers into the Z direction which is then packaged. Subsequently blowing (expanding) the product randomizes the X, Y and Z direction fibers to create random matrixes. The physical connections to build loft comes about as individual packets are expanded with multiple nodes within each packet. Loft comes about when each packet builds on one another with physical entanglements generated thru the expansion process making the connections between packets.

The invention provides:

a) a new product in the form of a blown-in insulated material made from short polymer fibers with respect to which several intermediate steps in the overall process give the final product key performance characteristics: b) the product is made by way of a modified melt blowing system with modifications providing higher levels of orientation and thermal stability to the fibers, small intermediate compressed packets for better handling and final low bulk density with high loft and high insulating value product; and c) new hardware adapted to work the molecules of the fiber to achieve the blown-in insulation product.

In order to maximize the properties of the fiber and the product (blown-in insulation) the new blown-in product has several steps by which it is formed.

The process comprises:

1) Fiber formation with a 1<sup>st</sup> orientation;

2) 2<sup>nd</sup> orientation of the fiber;

45 3) Redirection of some fibers to the Y direction, nodes created

4) Quench to lock in orientation

5) Additional crystallization to the fiber

6) Coating the fiber

7) 3rd orientation of fiber

8) Cutting fiber (multiple layers)

9) Compacted packets of fiber

10) Packaged (compressed) packets

55 11) Re-expanded fiber expands around nodes (and entanglements).

According to the invention there is provided a method of producing a non-lofted fiber veil of an orientable polymer for the production of insulation for blown-in applications having X, Y and Z vector directions of the fibers comprising: a) melt blowing the polymer to form molten fibers; b) using a high velocity air flow to orient molecules of the fibers along the length of the fibers, the X vector direction; c) placing the fibers on a mechanical roller adjacent the air flow which is spinning at a rate to provide additional orientation of the molecules of the fibers in the X vector direction as the fibers move across the air flow to the roller; d) using air flow turbulence and roller placement to displace some said fibers into

the Y vector direction; and e) cooling the roller to solidify the fibers while on the roller to form the non-lofted fiber veil.

More specifically according to the invention there is also provided a method of producing a non-lofted fiber veil of an orientable polymer for the production of insulation for blown-in applications having X, Y and Z vectors comprising: a) extruding the polymer by melt blowing to form molten fibers; b) directing a high velocity hot air flow around the extruded fibers with both the air flow and the length of the fibers having the same direction, the X vector direction, to carry the fibers in said direction and to orient the molecules of the fibers along the X vector direction of the fibers; c) locating a mechanical roller adjacent to the fibers being carried in said direction; d) placing the fibers on the roller which is spinning in a direction to carry the fibers away from the air flow; e) choosing a rate of rotation of the roller whereby force generated by the air flow pushing in said direction and the fibers moving across the air flow to the roller yields additional orientation of the molecules of the fibers in the X vector direction; f) placing the roller so that the placement of the roller and turbulence created by the air flow causes a percentage of the fibers to be displaced into a transverse direction, the Y vector; and g) cooling the roller to quench the fibers, after orientation of the molecules thereof subsequent to removal of the fibers from the air flow as they pass over the roller to prevent loss of orientation of the molecules, to form the non-lofted fiber veil.

Also a feature of the invention is the product of the methods of the previous two paragraphs.

Also according to the invention there is provided an apparatus for producing a non-lofted fiber veil of an orientable polymer for the production of insulation for blown-in applications having X, Y and Z vector directions of the fibers comprising: a) a melt blowing station for blowing the polymer to form molten fibers encompassed by using a high velocity air flow to orient molecules of the fibers along the length of the fibers, the X vector direction; b) a mechanical roller adjacent the air flow arranged to spin at a rate to provide additional orientation of the molecules of the fibers in the X vector direction as the fibers leave the air flow to reach to the roller; and together with air flow turbulence and placement of the roller, to displace some said fibers into the Y vector direction; and c) cooling means associated with the roller to solidify the fibers while on the roller to form the non-lofted fiber veil.

The invention further provides a non-lofted oriented polymer insulation for blown-in applications comprising multiple layers of oriented polymer veils compressed together and cut to form R-Buds of multiple layers of polymer fibers entangled and connected by nodes expandable upon installation to provide a blown-in insulation.

Also the invention provides an R-Bud for use in forming a matrix of insulation for blown-in applications of an orientable polymer comprising multiple superimposed layers of non-lofted veils, formed by fibers of said polymer disposed in both of X and Y vectors of X, Y and Z vectors, the veils being interconnected by fibers extending along the Z vector.

The invention also includes a blown-in insulation comprising a plurality of R-Buds according to the preceding paragraph each expanded to produce the insulation as a matrix of expanded R-Buds.

The invention further provides a method of producing a blown-in insulation from an orientable polymer comprising: a) producing a plurality of non-lofted veils each having a plurality of fibers of the polymer extending and interconnected in X and Y vectors of X, Y and Z vectors; b) superimposing the veils and compressing these together to produce interconnection of the layers along the Z vector; c) cutting the

interconnected layers into a plurality of R-Buds; and d) expanding the R-Buds, at the time of installation of the insulation, to form blown in insulation comprising a large plurality of the R-Buds.

#### BRIEF DESCRIPTION OF THE DRAWINGS

The invention will now be described, by way of example, with reference to the accompanying drawings in which:

10 FIG. 1 is a diagrammatic schematic of apparatus according to the invention also illustrating the steps of the method according to the invention;

15 FIG. 2 is a sketch showing the veil in the X and Y direction with node points 38 and 40 which continue to remain intact after cutting and compaction as shown in FIGS. 3-10; and

20 FIGS. 3-10 are diagrammatic sketches, micro-photographs and a drawing showing a combination of features all illustrating features of the blown and expanded R-Buds providing for their stable entanglement to provide a lofted insulation.

#### DESCRIPTION OF PREFERRED EMBODIMENTS

The apparatus illustrated in FIG. 1 comprises a melt blowing die apparatus 2 for melt blowing molten synthetic fibers entrained in a curtain 4 of air 6 emitted vertically at high speed parallel to the spun fibers at a temperature of about 600° F. ±100° F. The fibers extend primarily in an x direction and may comprise a polyester (i.e. PET) issuing from the nozzles of the apparatus 2 with a diameter of typically about 0.2 to 0.5 mm. These fibers are attenuated, oriented and fibrillated by the curtain of hot air to a statistical mean of about 5 to 15 microns (NOTE 1000 microns=1 mm) while at the same time molecular orientation takes place as the hot air quickly cools to an orientation temperature of about 200° F.

30 One of the major limitations to melt blowing in the prior art is that the hot air remains in contact with the fiber. The hot air keeps the fiber above Tg (glass transition temperature) which relaxes the molecules within the fiber thus reducing the orientation of the fiber. Better orientation can be achieved if the fiber after orientation is quenched. This locks in the orientation of the molecules otherwise orientation is lost through relaxation.

35 In view of this the fibers are removed from the air stream forming a loop 8 extending to a cold roller 10 rotating in the direction of arrow 12. The loop 8 provides a second orientation of the fibers which are then quenched on the roller 10 to lock in the orientation. At this stage the fibers form a substantially single layer web- or veil 14 with the majority of fibers in the x direction and some fibers extending in the Y direction of the veil comprising 10-20% of the fibers and with virtually no fibers extending in the Z direction (e.g. out of the plane of the

40 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 95

the mass of fibers will not collapse under its own weight. In turn, building a matrix of fine fibers allows a better insulating product as the matrix impedes the flow of air thus providing greater insulating value.

A characteristic of PET (and some other crystalline resins) is that it can be oriented which increases the crystallinity level via mechanical action but with PET one can also add crystallinity by way of adding thermal energy that allows crystals to grow. The term heat setting is used in the PET industry to describe crystalline growth through the addition of thermal energy. If the molecules are allowed to relax during heat setting then orientation will be lowered. With standard melt blowing, a good portion of the orientation is lost due to the thermal temperatures of the hot air used to draw the fiber, as the fiber is not restrained. In addition, exposure of the fiber to the hot air yields thermal crystallization. Thermal crystallization without good orientation yields a fiber that is brittle. In addition, the thermal relaxation of orientation causes the fiber diameter to increase as the 'memory' of the fiber tries to bring the fiber to its original (larger) fiber diameter. The increased thickness of the fiber is ineffective for insulation and filter products as it changes the bulk density of the final product.

Thus one or more veils 14 is then passed through a heat setting station 16 in which the veil 14 is restrained in both the X and Y directions to prevent shrinkage while being heated to crystallize the fibers using hot air represented by arrows 18. Other heating sources could be used i.e. infra red, radio frequency, etc. The restraint is shown diagrammatically at 20 and may comprise webs, plates, veil edge gripping devices, veil gripping porous conveyers etc.

Following heat setting additional veils 14 are added in overlapping manner to be fed together to a coating station 22 which may comprise coating rollers between which the multiple veils pass to be coated by a lubricant (i.e. a short chain polymer). The multiple veils leave the coating station still extending primarily only in the X and Y directions.

After coating the multiple veils are passed through a tow forming station 24 to a tow cutting station 26. The amount of coating can be used to control density in the final blown product. The tow is formed by pressing the multiple veils together in the Y direction to produce an overlapping fiber tow having X, Y and Z dimensions using control plates, rollers, etc. to produce a tow having substantially identical Y and Z dimensions. The cutting station 26 can operate faster than the supply rate of the veils supplied by the coating station 22 thereby cold drawing and further increasing molecular orientation of the fibers and decreasing their diameters.

The cutting station comprises a standard cutter unit which is adjusted as to speed and tension to cut the tow into compact R-Buds 28 of a desired tightness or density. The cutting operation also increases the proportion of fibers extending in the Z direction. The R-Buds are each of a basically rectangular packet configuration which are then compactly packaged at a packaging station 30 into bags for distribution to an end user.

The end user who is to install blown-in insulation may use a standard blown insulation installer 32 to expand the R-Buds 28 and add transport air to produce expanded packets of insulation from the R-Buds 28 which become entangled with one another to produce a stable lofted insulation 34 free of binders and brittle components coated only with a lubricant coating.

The lofted material is suitable not only for thermal but also sound insulation and is also useful as a fibration material among many other potential environmentally non-hazardous uses.

The re-expansion results in the actual installed product. The final bulk density can be controlled by the amount of mechanical action, velocity of air, coating material or coating amount. The expansion takes place when the R-Buds are put into a mechanical action machine which via a scouring action and the use of air to blow the product takes the compacted R-Buds and expands them into a product that is a 3 dimensional random matrix comprising fibers in equal proportion in the X, Y and Z directions. The bulk density can range from 0.25 to 2 lbs per cubic foot.

Typical Densities, in lb/cu.ft, of articles

Veil 0.8+/-0.1

R-Buds

12.5+/-5

15 Packaged R-Buds

17.5+/-5

Expanded

0.25-0.5

20 Standard mean fiber diameters from melt blowing operations range from 10 to 50 microns. In insulation, it is better to have smaller diameters but strong fibers. The range of fiber diameters for insulation products will vary depending on final application specifications but can generally be characterized into 2 groups; 1 to 10 micron average diameter and sub-micron 0.1 to 1 micron average. It has been found that for the blown-in insulation product a preferred statistical mean diameter should be in the 2 to 7 micron range.

25 The term density can apply to several areas. The individual fiber has a density that is often measured to calculate the degree of crystallization. The term bulk density is used to describe the density of the mass of fibers. For shipping and other purposes, a high bulk density is preferred so as to save space, freight, etc. When the product is used as an insulating material a low bulk density is preferred so as to be cost efficient. The blown-in insulation product also has a yield factor whereby the fiber diameter is critical to thermal insulation efficiency and cost. A smaller fiber diameter which for the same weight per given volume will yield more fibers thus better insulation than a larger diameter fiber.

30 For example a product may have the same fiber density and bulk density but very different yield with different fiber diameters. This yield is important to creating a matrix to trap airflow thus providing insulating value. Example: one fiber with a diameter of 0.015 mm and 10 mm long with a density of 1.35 grams/cc has a total mass of  $2.4 \times 10^{-6}$  grams. Using the same fiber density, mass and length and adjusting the diameter to 0.0075 mm (half the original) then 4 fibers can be made instead of the one. Nine (9) fibers can be made from the same mass if the diameter is adjusted to 0.005 mm (5 microns). [Note: 1.000 micron=1 mm)

35 Thus it is easily determined that the smaller fibers will give a more complex matrix if the fibers are suitably randomized in the X, Y and Z directions. Please note though, at average fiber diameters of less than 3 microns the fiber strength begins to become too weak to support itself in a stand-alone condition/position.

40 Referring now to FIGS. 2-10 various nodes and entanglement of the veil and expanded R-Buds 28 is illustrated with reference to the various mechanisms providing a stable lofted product. The redirected Y vector fiber is important to the final product. Interaction of the Y direction fibers with the X direction fibers is very important so as to create a 'veil' (web). This veil is made of X and Y fibers that hang together forming a web. The X and Y fibers hang together by several means. The intersections at which they meet are called nodes. These nodes can be formed by several means; entanglements (in-

cluding twistings) 38, friction/hang ups 40, welding 42, intermolecular attraction 44 due to polarity of the molecules, etc.

Entanglements are those fibers that wrap around another. Friction/hang ups are where the two fibers intersect and slide until caught at a node. This would be similar to a branch falling from a tree and getting caught in the limbs of a tree (where the limbs intersect the body or larger limb). Weld points are created when the hot fibers touch one another and then are frozen in place by the cold roller. Intermolecular attraction is present in several forms. When oriented a molecule will have a degree of polarity created. The opposite poles will attract and keep fibers together. Further, the fibers rubbing against one another creates static, which in turn, will keep the fibers bonded together.

The X direction fibers are more oriented than the Y direction fibers but even the Y vector fibers have a degree of orientation and thus have better strength than non-oriented fibers.

The micro-photographs of FIGS. 8, 9 and 10 illustrate the complexity of intermixed mechanisms controlling the stability of the lofted product after expansion.

The preferred insulation material is one that is composed of fibers that are thermally stable and have good strength and stiffness. Fibers that are weak will yield under a force. Fibers that are not thermally stable will collapse (due to gravitational force) or distort (shrinkage) upon exposure to elevated temperatures. Fibers that are brittle will break when exposed to any force. In turn, when the fibers are affected the entire insulation product is impacted thus the product fails.

A fiber that has good orientation and has been given thermal stability (such as heat setting) will provide a fiber that will make up a good insulation product.

| Orientation | Thermal Crystallization | Result                                                    |
|-------------|-------------------------|-----------------------------------------------------------|
| Low         | High                    | Brittle fiber                                             |
| Low         | Low                     | Product collapses when exposed to higher temps            |
| High        | Low                     | Product shrinks and distorts when exposed to higher temps |
| High        | High                    | Stable/strong product                                     |

The preferred method of the present invention comprises:

1. First orientation of fiber: Fiber formation has remained the same as described in previous patent applications assigned to the assignee of the present application. The fiber is extruded from a die which has a multitude of openings (holes, or the like) on the order of 0.5 mm in diameter. This hot extrudate is pushed out of the die hole and forms a molten fiber. High velocity air (e.g. hot for PET or cold for polypropylene) is directed around the newly formed fiber with both air and fiber directed in the same axis. (For this discussion; vertical direction) This air quickly carries the molten fiber downwardly and begins to orient the fiber;

2. Second orientation: Instead of keeping the fiber in the hot air until collected, a mechanical roller is located such that it is adjacent to the stream of fibers. See FIG. 1. The fibers are placed on the roller which is spinning. The downward force of the air orients the fiber. The preferred process is such that the fiber forms somewhat of an 'J' shape with a half loop at the bottom of the airflow. This force generated by the air pushing downwardly and the fiber trying to move across the airflow yield to produce more orientation as the fiber has restraints and cannot relax. This can be controlled by the vertical and horizontal position of the rollers.

3. Y direction: Due to the placement of the roller and the turbulence created by the flow of air a percentage of individual fibers are displaced into the Y vector. The % and diameters of the Y direction fibers can be managed by the 5 RPM and location of the roller relative to the fiber formation;

4. Quench: The rotating roller is cool to cold from internal cooling. This cold temperature quenches the oriented molecules in place. Further, the molecules are removed from the hot air to prevent relaxation (loss of orientation) of the molecules. The roller may be designed, i.e. as a corkscrew, to place the Y vector fibers in tension;

5. Added crystallization: Depending on the specifications, the fibers may need additional thermal crystallization once they have been orientated. To add thermal crystallization, the 15 fibers are restrained in both the X and Y directions while heat is applied. After sufficient time has elapsed to achieve desired crystallization the fibers have to be quenched while still restrained;

6. Coating: To enhance the cutting, compacting and re-expansion of the fibers, it is sometimes desirable to coat the fibers with a lubricant. This lubricant allows faster cutting and compaction and allows a lower installed density upon re-expansion of the fibers;

7. Third orientation: Third orientation of the fibers is performed when the fibers are put into the cutter (tow cutter) that can run at a higher speed than the roller feeding it. The fibers are cold drawn adding additional-orientation to the fiber;

8. Cutting: Cutting the fiber is accomplished by use of 30 device called a tow cutter. To get optimum performance, several veils are laid on top of one another and then bunched together to form a unit that is like a narrow non-woven rope. The bunching of the veils creates further complexion to the orientation of the fibers. Further entanglements form additional nodes. These bunched veils are cut into packets on the 35 order of 0.400 inches+/-0.300 inches in height;

9. Compacting: The fibers are purposely compacted in the tow cutter. This is accomplished by changing the machine process conditions so that discrete 3 dimensional rectangles with compacted fibers are formed. The compacted fibers are 40 formed into an R-Bud. The dimensions of the R-Bud are approximately 0.125 inch wide and 0.375 inch in depth. These packets (R-Buds) are loosely compacted such that friction or the like mechanical action will cause them to come apart. It should be noted that the R-Buds are formed from the 45 veil so that upon dissecting the R-Buds one finds portions of a mini-veil. The fibers are running in the X, Y and now Z directions relative to the R-Bud. The Z direction fibers are important to note as when the R-Bud is expanded into blown in insulation, the fibers then form a 3 dimensional matrix;

10. Packaging: For ease of shipment the R-Buds are packaged into a secondary package and some additional compression is added to increase the bulk density. This will ease the 50 cost of freight and handling; and

11. Expanding: Expanding the R-Buds via a machine that 55 will expand the R-Buds around the nodes and entanglements to produce a stable lofted product made up of a matrix of the expanded R-Buds, with superior insulating values due to the random 3D matrix of fibers created around the nodes.

---

Reference numerals

---

|   |                        |
|---|------------------------|
| 2 | melt blowing apparatus |
| 4 | curtain                |
| 6 | air                    |
| 8 | loop                   |

-continued

| Reference numerals |                      |
|--------------------|----------------------|
| 10                 | roller               |
| 12                 | arrow                |
| 14                 | veil                 |
| 16                 | heat setting station |
| 18                 | heat arrows          |
| 20                 | restraint            |
| 22                 | coating station      |
| 24                 | tow forming station  |
| 26                 | cutting station      |
| 28                 | R-Buds               |
| 30                 | packaging station    |
| 32                 | blow installer       |
| 34                 | lofted insulation    |
| 38                 | entanglement nodes   |
| 40                 | hang up nodes        |
| 42                 | welded nodes         |
| 44                 | static bond nodes    |

We claim:

1. A method of producing a substantially single layer non-lofted fiber veil of an orientable polymer for the production of insulation for a blown-in application having X, Y and Z vector directions, the method comprising steps of:
- extruding the polymer by melt blowing to form molten fibers;
  - directing a high velocity hot air flow around the extruded fibers with both the air flow and a length of the fibers having a common direction, the X vector direction, to carry the fibers in said X vector direction and to orient molecules of the fibers substantially along the X vector direction of the fibers;
  - locating a mechanical cold roller adjacent to the fibers being carried in said X vector direction, and the cold roller being spaced and offset from the high velocity hot air flow in the X vector direction such that the fibers are removed from the high velocity hot air flow by a removal loop, prior to the fibers engaging with the cold roller;
  - placing the fibers on the cold roller which is spinning in a direction to carry the fibers further away from the air flow in the X vector direction;
  - choosing a rate of rotation of the cold roller whereby a force generated by the air flow pushing in said X vector direction and the fibers moving across the air flow in the removal loop toward the cold roller yields additional orientation of the fibers in the X vector direction;
  - placing the cold roller so a placement of the cold roller and turbulence created by the air flow causes a percentage of the fibers to be displaced into a transverse Y vector direction;
  - heat setting the non-lofted fiber veil by restraining the veil formed in step f) in both the X and Y vector directions, heating the restrained veil for a period of time and at a temperature to produce desired crystallinity of the fibers of the veil;
  - cooling the cold roller to quench the extruded fibers, after orientation of the molecules thereof and subsequent to removal of the fibers from the air flow, as the fibers pass over the cold roller to prevent loss of orientation of the molecules and form the substantially single layer non-lofted fiber veil and;
  - applying tension to the substantially single layer non-lofted fiber veil, prior to cutting the substantially single layer non-lofted fiber veil, to facilitate further alignment of the fibers in the X vector direction and minimize any alignment of the fibers in the Y and Z vector directions.
2. The method of claim 1 further comprising the step of heat setting the non-lofted fiber veil by restraining the veil formed in step f) in both the X and Y vector directions, heating the restrained veil for a period of time and at a temperature to
- produce a desired crystallinity of the fibers of the veil, and quenching the heated veil while still restrained.
- The method of claim 2 further comprising the step of coating the fibers of the crystallized and quenched veil with a lubricant to facilitate faster cutting and compaction and provide for a lower installed density, upon expansion of a blown in insulation formed from a plurality of the veils.
  - The method of claim 1 further comprising the step of cutting the veil in a tow cutter into a plurality of R-Buds having a height of about 0.4 inches (10 mm) +/- 0.3 inches (8 mm).
  - A method of producing a substantially single layer non-lofted fiber veil of an orientable polymer for the production of insulation for a blown-in application having X, Y and Z vector directions, the method comprising the steps of:
    - extruding the polymer by melt blowing to form extruded fibers;
    - directing a high velocity hot air flow around the extruded fibers with both the air flow and a length of the fibers having a common direction, the X vector direction, to carry the fibers in the X vector direction and to orient molecules of the fibers along the X vector direction of the extruded fibers;
    - locating a mechanical cold roller adjacent to the extruded fibers being carried in the X vector direction such that the fibers are removed from the high velocity hot air flow by a removal loop, prior to the fibers engaging with the cold roller;
    - placing the extruded fibers on the cold roller which is spinning so as to carry the fibers away from the air flow;
    - choosing a rate of rotation of the cold roller whereby a force generated by the air flow pushing in the X vector direction and the fibers moving across the air flow in the removal loop toward the cold roller yields additional orientation of the molecules of the fibers in the X vector direction;
    - placing the cold roller so that the placement of the cold roller and turbulence created by the air flow causes a percentage of the fibers to be displaced into a transverse Y vector direction;
    - heat setting the non-lofted fiber veil by restraining the veil formed in step f) in both the X and Y vector directions, heating the restrained veil for a period of time and at a temperature to produce desired crystallinity of the fibers of the veil;
    - cooling the cold roller to quench the extruded fibers, after orientation of the molecules thereof and subsequent to removal of the fibers from the air flow as the fibers pass over the cold roller to prevent loss of orientation of the molecules and form the substantially single layer non-lofted fiber veil;
    - applying tension to the substantially single layer non-lofted fiber veil, prior to cutting the substantially single layer non-lofted fiber veil, to facilitate further alignment of the fibers in the X vector direction and minimize any alignment of the fibers in the Y and Z vector directions prior to cutting the substantially single layer non-lofted fiber veil in a tow cutter; and
    - laying a plurality of the veils on top of one another and compressing the plurality of the veils together to form a non-woven multi-layer structure of fibers having substantially most of the fibers extending in the X vector direction.

6. The method of claim 5 further comprising the step of mechanically bunching the veils together to form entanglements and nodes in addition to those formed in prior steps of the method.

**11**

7. The method of claim **5** further comprising the step of cutting the bunched veils to form R-Buds of about 0.4 inches (10 mm) +/-0.3 inches (8 mm) in height.

8. The method of claim **5** further comprising the step of compacting the bunched veils so that the bunched veils have X, Y and Z dimensions, and cutting the compacted veils to form three dimensional R-Buds having fibers extending substantially in the X vector direction.

9. The method of claim **8** wherein the R-Buds are about 0.125 inches (3 mm) wide and about 0.375 inches (10 mm) in depth with the R-Buds being loosely compacted such that mechanical action will cause the R-Buds to separate and come apart.

10. The method of claim **9** further comprising the step of compressing and packaging the R-Buds into a secondary package to increase the bulk density and thereby to reduce the cost of freight and handling.

11. The method of claim **9** further comprising the step of expanding the R-Buds around nodes and entanglements in the R-Buds to produce blown-in insulation in a stable lofted form.

12. The method of claim **1** wherein said X vector direction is vertically downward.

13. The method of claim **1** wherein the molten fibers in the melt blowing step are about 0.02 inches (0.5 mm) in diameter.

14. The method of claim **1** wherein the periphery of the cold roller is shaped to facilitate displacement of fibers into the Y vector direction.

**12**

15. A method of producing an insulation for blown-in applications from an orientable polymer, the method comprising the steps of:

- a) producing a plurality of non-lofted veils, each of the plurality of non-lofted veils being substantially a single layer having a plurality of fibers of the polymer extending substantially in the X vector direction and engaging each substantially single layer non-lofted veil with a cold roller, following formation thereof, to quench the fibers of the polymer and prevent loss of molecule orientation, the cold roller being spaced and offset from a high velocity hot air flow in the X vector direction such that the fibers are removed from the high velocity hot air flow by a removal loop, prior to the fibers engaging with the cold roller, such that the fibers moving across the air flow in the removal loop toward the cold roller yields additional orientation of the fibers in the X vector direction;
- b) superimposing the substantially single layer non-lofted veils and compressing the substantially single layer non-lofted veils together to produce interconnection of the layers along a Z vector;
- c) cutting the interconnected layers into a plurality of R-Buds having a height of about 0.4 inches (10 mm) +/-0.3 inches (8 mm); and
- d) expanding and separating the R-Buds into discrete fibers, at the time of installation of the insulation, to form blown in insulation comprising a 3 dimensional random matrix of discrete fibers.

\* \* \* \* \*